# EUROPEAN PATENT SPECIFICATION

(11) **EP 3 124 645 B1**
(45) Date of publication and mention of the grant of the patent: **23.10.2019**
(21) Application number: 14887198.1
(22) Date of filing: 17.12.2014
(51) Int. Cl.: C23C 8/14, C23C 8/80, C21D 9/14, C22C 30/00, C22C 38/00, C22C 38/02, C22C 38/04, C22C 38/06, C22C 38/44, C22C 38/48, C22C 38/50, C22C 38/54, C22C 19/05

(54) **CASTING PRODUCT HAVING ALUMINA BARRIER LAYER**
GIESSPRODUKT MIT ALUMINIUMOXIDSPERRSCHICHT
PRODUIT DE FONDERIE AYANT UNE COUCHE BARRIÈRE EN ALUMINE

(30) Priority: 28.03.2014 JP 2014067836
(43) Date of publication of application: 01.02.2017
(73) Proprietor: Kubota Corporation, Osaka-shi, Osaka 556-8601 (JP)
(72) Inventor: HASHIMOTO Kunihide, Hirakata-shi Osaka 573-8573 (JP); URAMARU Shinichi, Hirakata-shi Osaka 573-8573 (JP)
(74) Representative: Ter Meer Steinmeister & Partner
(86) International application number: PCT/JP2014/083417
(87) International publication number: WO 2015/145896

(56) References cited:
- WO-A1-2012/054377
- CA-A1- 2 868 306
- JP-A- S5 331 517
- JP-A- H05 195 138
- JP-A- S54 125 118
- JP-A- 2007 119 802
- JP-A- 2013 199 672
- JP-A- 2013 227 655
- JP-A- 2014 501 620
- US-A- 4 248 629
- US-A1- 2009 314 390
- US-A1- 2011 318 593
- SADAO OTA ET AL.: 'Effect of addition of Al, Zr, Y, Ce, La and Hf on the carburization resistance of high-Si-25Cr-35Ni alloy' JOURNAL OF THE IRON & STEEL INSTITUTE OF JAPAN vol. 67, no. 13, 10 September 1981, page 1266, XP055356070

## Description

### BACKGROUND OF THE INVENTION

### Field of the Invention

The present invention relates to a cast product having an alumina barrier layer, and more specifically, to a cast product having an alumina barrier layer with a stable structure.

### Description of the Related Art

Heat-resistant steel castings such as reaction tubes and decomposition tubes for producing ethylene, and hearth rolls, radiant tubes and metal dusting-resistant materials for use in carburizing heat-treatment furnaces are exposed to a high-temperature atmosphere, and therefore are made of an austenite-based heat-resistant alloy having superior high-temperature strength.

A metal oxide layer is formed on the surface of this type of austenite-based heat-resistant alloy during use in a high-temperature atmosphere. This oxide layer serves as a barrier, and thus protects the base material under a high-temperature atmosphere.

On the other hand, when Cr-oxides (mainly constituted by Cr₂O₃) are formed as the metal oxide, the Cr-oxide layer has an insufficient function for preventing the entry of oxygen and carbon due to its low denseness, thus causing the internal oxidation under a high-temperature atmosphere and the thickening of the oxide film. Moreover, the Cr-oxide layer is likely to become detached during repeated cycles of heating and cooling. Even if the Cr-oxide layer do not become detached, the Cr-oxide layer has an insufficient function for preventing the entry of oxygen and carbon from an outside atmosphere, and therefore, there is a disadvantageous situation in which oxygen and carbon pass through the film and cause the internal oxidation or carburization of the base material.

To address this, it is proposed that an oxide layer including alumina (Al₂O₃) as a main component that has high denseness and makes it difficult for oxygen and carbon to pass therethrough is formed on the surface of the base material by increasing the content of Al compared with that in a common austenite-based heat-resistant alloy (see Patent Documents 1 and 2, for example).

However, Al is a ferrite-forming element, and therefore, when the content of Al is increased, the ductility of the materials is deteriorated and the high-temperature strength is reduced. This tendency of reduction of the ductility is observed particularly when the content of Al exceeds 5%

For this reason, the austenite-based heat-resistant alloy of Patent Documents 1 and 2 can be expected to have an enhanced barrier function due to Al₂O₃, but has the disadvantage of causing a reduction of the ductility of the base material.

Therefore, in order to provide a cast product that can secure the high-temperature stability of Al₂O₃ and can achieve a superior barrier function under a high-temperature atmosphere without reducing the ductility of the materials, Patent Document 3 proposes a cast product in which an alumina barrier layer including Al₂O₃ is formed on the inner surface of a cast body and Cr-based particles that contain Cr at a higher concentration than that of a matrix of the base material are dispersed at an interface between the alumina barrier layer and the cast body by performing heat treatment under an oxidizing atmosphere after processing the inner surface such that a surface roughness (Ra) of the cast body is 0.05 to 2.5 µm (see Patent Document 3, for example).

Due to the presence of a stable alumina barrier layer, superior oxidation resistance, carburization resistance, nitriding resistance, corrosion resistance, and the like of the cast product of Patent document 3 can be maintained for a long period of time of use under a high-temperature atmosphere.

### PRIOR ART DOCUMENTS

### PATENT DOCUMENTS

Patent Document 1: JP S52-78612A
Patent Document 2: JP S57-39159A
Patent Document 3: WO 2010/113830

US 2011/318593 A1 (Takahashi Makoto [JP] et al.) relates to a cast product comprising a cast body of a heat-resistant alloy comprising of, in mass percent, 0.05 to 0.7% of C, over 0% to up to 2.5% of Si, over 0% to up to 3.0% of Mn, 15 to 50% of Cr, 18 to 70% of Ni, 2 to 4% of Al, 0.005 to 0.4% of rare-earth elements, and 0.5 to 10% of W and/or 0.1 to 5% of Mo, the balance being Fe and inevitable impurities, and a barrier layer formed at a surface of the cast body to be brought into contact with said high temperature atmosphere, said barrier layer comprising an Al₂O₃ layer having a thickness of 0.5 µm or more wherein at least 80 area % of the outermost surface thereof is Al₂O₃.

JP 2007 119 802 A (Central Res Inst Elect) relates to a heat-resistant metallic material composed of an aluminum-containing nickel-based alloy wherein the resistant metallic material is obtained by a heat-treatment in a low oxygen partial pressure atmosphere.

It is an object of the present invention to provide a cast product that can further enhance the stability of the alumina barrier layer and can exhibit further superior oxidation resistance, carburization resistance, nitriding resistance, corrosion resistance, and the like when used under a high-temperature atmosphere.

### SUMMARY OF THE INVENTION

The cast product as described herein is a cast product having an alumina barrier layer including an aluminum oxide on a surface of a matrix, wherein the aluminum oxide is (Al₍₁₋ₓ₎M₍ₓ₎)₂O₃, where M is at least one of Cr, Ni, Si, and Fe, and x satisfies a relationship 0<x<0.5.

Also, the cast product according to the present invention is a cast as defined in claim 1.

### EFFECTS OF THE INVENTION

With the cast product of the present invention, at least one of Cr, Ni, Si, and Fe forms a solid solution in an alumina barrier layer formed on a surface of a matrix, thus enabling an aluminum oxide phase to have a stable structure. With the aluminum oxide, it is possible to suppress the coupling between the matrix and oxygen and the formation of oxides containing Cr, Ni, Si, Fe and the like as a main component on the surface of the matrix.

This makes it possible that the cast product of the present invention exhibits further superior oxidation resistance, carburization resistance, nitriding resistance, corrosion resistance, and the like when used under a high-temperature atmosphere.

Accordingly, when the cast product of the present invention is used for a reaction tube for producing ethylene, for example, it is possible to suppress the occurrence of coking, to prevent the yield from being reduced by the reduction of heat exchange rate and thermal conductivity due to the occurrence of coking, and to extend continuous operating time. In addition, since coking is unlikely to occur, it is possible to reduce the frequency and time period for coking-removing operation and to enhance operation efficiency.

### BRIEF DESCRIPTION OF THE DRAWINGS

FIG. 1 is a cross-sectional view of a cast product before heat treatment.
FIG. 2 is a schematic cross-sectional view illustrating a state where a dilute-Al layer is formed by low-temperature heat treatment.
FIG. 3 is a schematic cross-sectional view illustrating a state where a concentrated-Al layer is formed between the dilute-Al layer and a matrix by high-temperature heat treatment.
FIG. 4 shows a TEM photograph of a film of Working Example 2 and graphs illustrating the results of an EDX analysis.
FIG. 5 shows a TEM photograph of a film of Working Example 7 and graphs illustrating the results of an EDX analysis.

### DESCRIPTION OF THE PREFERRED EMBODIMENTS

Hereinafter, embodiments of the present invention will be described in detail.

A cast product of the present invention has an alumina barrier layer including an aluminum oxide on the surface of a matrix.

Also, at least one of Cr, Ni, Si, and Fe forms a solid solution in the aluminum oxide in the alumina barrier layer, and at least one of Cr, Ni, Si, and Fe forming a solid solution with Al is contained so as to satisfy the relationship Al/(Cr+Ni+Si+Fe)≥2.0 in an atomic % ratio.

### Explanation of reasons for limiting components

As long as the cast product of the present invention is made of a heat-resistant alloy containing Cr in an amount of 15 mass% or more, Ni in an amount of 18 mass% or more, and Al in an amount of 1 to 5 mass%, it is possible to obtain the effects of the present invention. The cast product of the present invention is made of the following components. It should be noted that in the following description, the term "%" refers to "mass%" unless otherwise stated.

### C: 0.05 to 0.7%

C acts to improve castability and enhance a high-temperature creep rupture strength. Therefore, the content of C is set to at least 0.05%. However, if the content is too large, a primary carbide of Cr₇C₃ is likely to be extensively formed and the movement of Al for forming the alumina barrier layer is suppressed. As a result, Al is insufficiently supplied to the surface portion of a cast body and the alumina barrier layer is locally divided, and thus the continuity of the alumina barrier layer is impaired. Moreover, a secondary carbide excessively deposits to reduce ductility and toughness. Therefore, the upper limit is set to 0.7%. It should be noted that the content of C is more desirably 0.3 to 0.5%.

### Si: more than 0% to 2.5% or less

Si is contained to serve as a deoxidizer for molten alloy and to enhance the fluidity of molten alloy. If the content is too large, a high-temperature creep rupture strength is reduced, and therefore, the upper limit is set to 2.5%. It should be noted that the content of Si is more desirably 2.0% or less.

### Mn: more than 0% to 3.0% or less

Mn is contained to serve as a deoxidizer for molten alloy and to fix S in molten alloy. If the content is too large, high-temperature creep rupture strength is reduced, and therefore, the upper limit is set to 3.0%. It should be noted that the content of Mn is more desirably 1.6% or less.

### Cr: 15.0 to 50.0%

Cr is contained in an amount of 15.0% or more in order to contribute to the enhancement of high-temperature strength and cyclic oxidation resistance. However, if the content is too large, high-temperature creep rupture strength is reduced, and therefore, the upper limit is set to 50.0%. It should be noted that the content of Cr is more desirably 23.0 to 35.0%.

### Ni: 18.0 to 70.0%

Ni is an element that is necessary to secure cyclic oxidation resistance and the stability of a metal structure. If the content of Ni is small, the content of Fe relatively becomes large. As a result, a Cr-Fe-Mn oxide is likely to be formed on the surface of the cast body, and thus the formation of the alumina barrier layer is inhibited. Therefore, the content of Ni is set to at least 18.0%. Even if the content of Ni exceeds 70.0%, it is impossible to obtain the efficacy corresponding to the increasing amount, and therefore, the upper limit is set to 70.0%. It should be noted that the content of Ni is more desirably 28.0 to 45.0%.

### Al: 1.0 to 5.0%

Al is an element that is effective for enhancing carburization resistance and coking resistance. Also, in the present invention, Al is an element that is essential for forming the alumina barrier layer on the surface of the cast body. Therefore, the content of Al is set to at least 1.0%. However, if the content of Al exceeds 5%, the ductility is deteriorated, and therefore, the upper limit is set to 5.0% in the present invention. It should be noted that the content of Al is more desirably 2.5 to 3.8%.

### Rare earth elements: 0.005 to 0.4%

The term "rare earth elements" means 17 elements including 15 elements of the lanthanide series ranging from La to Lu in the periodic table, and Y and Sc. It is preferable that rare earth elements to be contained in the heat-resistant alloy of the present invention include at least one element selected from the group consisting of Ce, La and Nd. Rare earth elements contribute to the formation of the alumina barrier layer and the enhancement of stability thereof.

When the alumina barrier layer is formed by heat treatment under a high-temperature oxidizing atmosphere, rare earth elements that are contained in an amount of 0.005% or more effectively contribute to the formation of the alumina barrier layer.

On the other hand, if the content is too large, the ductility and toughness are deteriorated, and therefore, the upper limit is set to 0.4%.

### W: 0.5 to 10.0% and/or Mo: 0.1 to 5.0%

W and Mo enhance creep rupture strength by forming a solid solution in a matrix and strengthening an austenite phase. At least one of W and Mo is contained in order to achieve this efficacy. The content of W is set to 0.5% or more, and the content of Mo is set to 0.1% or more.

However, if the contents of W and Mo are too large, ductility is reduced and carburization resistance is deteriorated. Moreover, as in the case where the content of C is large, a primary carbide of (Cr, W, Mo)₇C₃ is likely to be extensively formed and the movement of Al for forming the alumina barrier layer is suppressed. As a result, Al is insufficiently supplied to the surface portion of the cast body and the alumina barrier layer is locally divided, and thus the continuity of the alumina barrier layer is likely to be impaired. Furthermore, since W and Mo have a large atomic radius, they suppress the movement of Al and Cr and inhibit the formation of the alumina barrier layer due to the formation of a solid solution in the matrix.

Therefore, the content of W is set to 10.0% or less, and the content of Mo is set to 5.0% or less. It should be noted that when both elements are contained, the total content is preferably set to 10.0% or less.

In addition, the following components are contained.

At least one selected from the group consisting of Ti in an amount of 0.01 to 0.6%, Zr in an amount of 0.01 to 0.6%, and Nb in an amount of 0.1 to 1.8%

Ti, Zr and Nb are elements that are likely to form carbides, and form less solid solutions in the matrix than W and Mo. Therefore, Ti, Zr and Nb do not exhibit any particular action of forming the alumina barrier layer, but enhance creep rupture strength. At least one of Ti, Zr and Nb can be contained as needed. The content of Ti or Zr is set to 0.01% or more and the content of Nb is set to 0.1% or more.

However, if they are excessively added, ductility is reduced. Furthermore, Nb reduces the peeling resistance of the alumina barrier layer. Therefore, the upper limit of the content of Ti or Zr is set to 0.6%, and the upper limit of the content of Nb is set to 1.8%.

### B: 0% to 0.1%

Since B exhibits an action of strengthening the particle boundaries of the cast body, B can be contained as needed. It should be noted that if the content of B is large, creep rupture strength is reduced, and therefore, the content of B is set to 0.1% or less even in the case where B is added.

The heat-resistant alloy making up the cast body of the present invention includes the above-described components and Fe as the balance. P, S, and other impurities that are inevitably mixed in the alloy when melting the alloy may be contained as long as such impurities are contained in an amount within a range that is usually allowable to this type of alloy material.

### Cast product

Molten metal having a composition including the above-described components is produced and cast by centrifugal casting, static casting, or the like into the cast product of the present invention having the above composition.

The obtained cast product can be shaped depending on the intended application.

One example of the cast product is a tube, in particular, a reaction tube used under a high-temperature environment.

It is particularly preferable to produce the cast product of the present invention by centrifugal casting. This is because when using centrifugal casting, a fine metal structure grows in the radial direction with orientation due to the progress of cooling by a metal mold and thus an alloy structure in which Al easily moves can be obtained.

Heat treatment, which will be described later, is performed on the cast product. The alumina barrier layer having a stable phase structure is formed by the heat treatment.

### Heat treatment

The heat treatment is performed on the cast product of the present invention under an oxidizing atmosphere. The heat treatment is divided into low-temperature heat treatment and high-temperature heat treatment. It should be noted that the low-temperature heat treatment and the high-temperature heat treatment can be performed in separate steps or the high-temperature heat treatment may be performed subsequently to the low-temperature heat treatment.

### Low-temperature heat treatment

The low-temperature heat treatment is treatment in which an aluminum oxide layer is formed on the surface of the matrix under an oxidizing atmosphere. The low temperature is 600 to 900°C. It is to perform the low-temperature heat treatment for 5 to 15 hours.

By performing the low-temperature heat treatment, oxygen comes into contact with a matrix 10 as shown in FIG. 1 to oxidize Al, Cr, Ni, Si, and Fe that has diffused from the matrix 10 to the surface of the matrix, and an oxide layer 22 is formed as shown in FIG. 2. Since this heat treatment is performed at a low temperature, Al forms oxides prior to Cr, Ni, Si, and Fe. Accordingly, an aluminum oxide layer 22 that contains Al as a main component and in which at least one of Cr, Ni, Si, and Fe, which have similarly diffused from the matrix, forms a solid solution is the oxide layer.

In the aluminum oxide formed by the low-temperature heat treatment, at least one of Cr, Ni, Si, and Fe forming a solid solution with Al is contained so as to satisfy the relationship Al/(Cr+Ni+Si+Fe)≥2.0 in an atomic % ratio. In addition, it is desirable that the composition thereof is (Al₍₁₋ₓ₎M₍ₓ₎)₂O₃, where M is at least one of Cr, Ni, Si, and Fe, and x satisfies the relationship 0<x<0.5. Moreover, at least Cr forms a solid solution in the aluminum oxide, and Cr forming a solid solution with Al is more preferably contained so as to satisfy the relationship Al/Cr≥10 in atomic % ratio, and still more preferably the relationship Al/Cr≥15. Furthermore, at least one of Ni, Si, and Fe forms a solid solution, and it is more desirable that the total atomic % of at least one of Ni, Si, and Fe forming a solid solution with Al is 10 atm% or less.

The aluminum oxide formed by the above-described low-temperature heat treatment has a metastable γ or θ alumina structure, which is a porous structure. Accordingly, the strength is not enough.

### High-temperature heat treatment

The high-temperature heat treatment is heat treatment that is performed after the low-temperature heat treatment, and in which, as described later, the phase of the aluminum oxide formed by the low-temperature heat treatment is transformed to an α alumina structure (corundum structure), and an aluminum oxide layer containing Al at a high concentration is formed between that aluminum oxide layer and the matrix.

The high-temperature heat treatment is performed by heating the cast product on which the low-temperature heat treatment has been performed and the alumina barrier layer having a γ or θ alumina structure has been formed, at a high temperature under an oxidizing atmosphere. The high temperature is a temperature of 1050°C or more. It is to perform the high-temperature heat treatment for 3 to 15 hours.

By performing the high-temperature heat treatment, the phase of the aluminum oxide that was formed first and has a γ or θ alumina structure is transformed to a stable α alumina structure (corundum structure). In the present invention, at least one of Cr, Ni, Si, and Fe forms a solid solution in the aluminum oxide layer having a γ or θ alumina structure. This makes it possible to promote the phase transformation from a γ or θ alumina structure to an α alumina structure (corundum structure) compared with the case where the aluminum oxide layer contains Al in a high ratio.

Then, the high-temperature heat treatment is further continuously performed on the cast product having the aluminum oxide layer in which the phase has been transformed to an α alumina structure (corundum structure), and thus oxygen passes through the aluminum oxide layer 22 as shown in FIG. 3.

The oxygen that has passed through the aluminum oxide layer 22 oxidizes Al that diffuses from the matrix, and an aluminum oxide layer 24 that contains Al at a high concentration is formed.

Here, as shown in FIG. 3, the aluminum oxide layer that is formed by the low-temperature heat treatment and in which at least one of Cr, Ni, Si, and Fe forms a solid solution is referred to as "dilute-Al layer", and the aluminum oxide layer that is formed between the dilute-Al layer and the surface of the matrix and contains Al at a high concentration is referred to as "concentrated-Al layer". Specifically, in the concentrated-Al layer 24, Al/(Cr+Ni+Si+Fe) is larger than that in the dilute-Al layer 22.

It is thought that the reason why in terms of the alumina barrier layer, the concentrated-Al layer formed between the matrix and the dilute-Al layer contains Al at a higher concentration than the dilute-Al layer at the surface is as follows.

The formed dilute-Al layer 22 allows a small amount of oxygen to pass therethrough under an oxidizing atmosphere.

Al, Cr, Ni, Si, and Fe diffuse from the matrix 10 side to the matrix surface side as shown in FIG. 3. However, since Al needs a smaller amount of energy for binding to oxygen than Cr, Ni, Si, and Fe, Al priorly binds to oxygen, and the aluminum oxide layer (concentrated-Al layer 24) containing aluminum oxide at a high concentration is formed between the matrix 10 and the dilute-Al layer 22.

The concentrated-Al layer 24 is formed by high-temperature heat treatment, and thus has a stable α alumina structure (corundum structure). It is desirable that 80 vol% or more of a crystal structure of each of the dilute-Al layer 22 and the concentrated-Al layer 24 is an α alumina structure (corundum structure).

Since the alumina barrier layer 20 is constituted by the dilute-Al layer 22 and the concentrated-Al layer 24 formed between the matrix 10 and the dilute-Al layer 22, both of which have stable α alumina structures (corundum structures), the alumina barrier layer 20 has high denseness, serves as a barrier for preventing oxygen, carbon and nitrogen from entering the base material from the outside during use under a high-temperature atmosphere in the cast product provided therewith, and can maintain superior oxidation resistance, carburization resistance, nitriding resistance, corrosion resistance, and the like for a long period of time.

It should be noted that the concentrated-Al layer 24 is desirably formed so as to be thicker than the dilute-Al layer 22, and it is preferable to form the concentrated-Al layer 24 such that the thickness of the concentrated-Al layer 24 is one fifth or more of that of the alumina barrier layer 20.

It is more desirable that the dilute-Al layer 22 has a thickness of 0.04 to 8.0 µm and the concentrated-Al layer 24 has a thickness of 0.01 to 2.0 µm.

It is desirable to heat the cast product while rotating it in order to preferably form the aluminum oxide layer in the above-described low-temperature heat treatment and high-temperature heat treatment. This makes it possible to heat the cast product uniformly and bring the cast product into contact with oxygen in a good state. As a result, it is possible to reduce the surface roughness (Ra) of the formed alumina barrier layer 20.

### Surface treatment

It is possible to perform surface treatment on the alumina barrier layer of the cast product as needed. One example of the surface treatment is polishing. For example, when the cast product is used for a reaction tube, Fe, Ni and the like of the cast product come into contact with a hydrocarbon as a raw material and coke (carbon) is likely to adhere to the inner surface of the tube due to the catalytic action of Fe and Ni, but it is possible to suppress the adhesion of coke by performing the surface treatment to reduce the surface roughness (Ra) of the alumina barrier layer.

It is desirable to perform the surface treatment such that the surface roughness (Ra) of the alumina barrier layer is 15 µm or less. The surface roughness (Ra) is more desirably 0.05 to 10 µm.

### Example 1

Molten metal was produced by atmospheric melting in a highfrequency induction melting furnace and cast by metal mold centrifugal casting into tube bodies having alloy chemical compositions shown in Table 1 below. The tube body has an inner diameter of 80 mm, an outer diameter of 100 mm, and a length of 250 mm.

**Table 1**

| No. | Alloy chemical composition (the balance includes Fe and inevitable im purities) (mass%) | | | | | | | | | | | | |
|---|---|---|---|---|---|---|---|---|---|---|---|---|---|
| | C | Si | Mn | Cr | Ni | Al | REM | W | Mo | Ti | Zr | Nb | B |
| Work. Ex. 1 | 0.33 | 0.49 | 0.32 | 24.5 | 43.6 | 1.2 | 0.25 | 2.1 | | 0.6 | | 0.7 | |
| Work. Ex. 2 | 0.45 | 0.49 | 0.9 | 24.3 | 34.6 | 1.0 | 0.16 | | 1.5 | 0.13 | | | |
| Work. Ex. 3 | 0.4 | 0.33 | 0.7 | 23.8 | 31.5 | 3.3 | 0.26 | | 2.8 | | | | 0.03 |
| Work. Ex. 4 | 0.46 | 1.5 | 1.2 | 25.2 | 35.0 | 2.8 | 0.21 | 4.2 | | 0.09 | 0.12 | | |
| Work. Ex. 5 | 0.26 | 0.41 | 0.5 | 23.5 | 34.6 | 3.1 | 0.07 | 0.9 | | | | | 0.07 |
| Work. Ex. 6 | 0.31 | 0.4 | 0.2 | 18.3 | 67.1 | 4.7 | 0.01 | | 0.4 | | | 1.6 | |
| Work. Ex. 7 | 0.38 | 0.26 | 0.4 | 23.8 | 34.4 | 4.9 | 0.11 | 0.95 | | | | 0.1 | |
| Work. Ex. 8 | 0.67 | 1.5 | 1.1 | 23.9 | 40.1 | 4.9 | 0.19 | | 2.9 | 0.03 | | | |
| Comp. Ex. 1 | 0.33 | 1.78 | 0.17 | 25.0 | 33.4 | 0.0 | 0.11 | 0.83 | | 0.12 | | | |
| Comp. Ex. 2 | 0.40 | 1.3 | 0.9 | 25.4 | 15.0 | 0.9 | 0.29 | 2.9 | | | | | |
| Comp. Ex. 3 | 0.27 | 1.02 | 0.2 | 23.8 | 33.6 | 1.1 | 0.19 | 11.7 | | | | | |
| Comp. Ex. 4 | 0.34 | 0.6 | 0.2 | 25.0 | 45.4 | 2.9 | 0.09 | | 1.5 | | | 1.3 | |
| Comp. Ex. 5 | 0.45 | 1.43 | 1.3 | 22.9 | 34.7 | 3.2 | 0.24 | 3.15 | | 0.23 | | | |
| Comp. Ex. 6 | 0.45 | 0.54 | 0.7 | 23.8 | 29.7 | 5.1 | 0.15 | 1.5 | | 0.21 | | | |

Two steps of heat treatment that differed in a heating temperature were performed on each of Working Examples 1 to 8, which were obtained examples of the present invention, and Comparative Examples 1 to 6 under an oxidizing atmosphere. First, the low-temperature heat treatment was performed, and the high-temperature heat treatment was subsequently performed. The low-temperature heat treatment was performed for 5 hours, and the high-temperature heat treatment was performed for 5 hours.

**Table 2**

| No. | Low-temperature heat treatment temperature (°C) | High-temperature heat treatment temperature (°C) |
|---|---|---|
| Work. Ex. 1 | 700 | 1050 |
| Work. Ex. 2 | 900 | 1100 |
| Work. Ex. 3 | 800 | 1050 |
| Work. Ex. 4 | 800 | 1100 |
| Work. Ex. 5 | 900 | 1100 |
| Work. Ex. 6 | 600 | 1050 |
| Work. Ex. 7 | 700 | 1100 |
| Work. Ex. 8 | 600 | 1150 |
| Comp. Ex. 1 | 800 | 900 |
| Comp. Ex. 2 | 1000 | 1250 |
| Comp. Ex. 3 | 1200 | 1300 |
| Comp. Ex. 4 | 500 | 1150 |
| Comp. Ex. 5 | 900 | 1000 |
| Comp. Ex. 6 | 600 | 800 |

The atomic percentages of elements (Al, Cr, Fe, Ni, Si, O) contained in the alumina barrier layer formed on the surface of a sample tube of each of Working Examples 1 to 8 and Comparative Examples 1 to 6 that had been subjected to the heat treatment were measured by an EDX analysis (energy dispersive X-ray spectrometry). Table 3 shows the results.

**Table 3**

| No. | Al (atm%) | Cr (atm%) | Fe (atm%) | Ni (atm%) | Si (atm%) | O (atm%) | Cr+Fe +Ni+Si (atm%) | Al/ (Cr+Fe +Ni+Si) | Al/Cr | Fe+Ni +Si (atm%) | Concentrated-Al layer thickness /Al barrier layer thickness |
|---|---|---|---|---|---|---|---|---|---|---|---|
| Work. Ex. 1 | 41.66 | 2.7 | 4.46 | 3.52 | | 48.56 | 10.7 | 3.9 | 15.43 | 7.98 | 0.50 |
| Work. Ex. 2 | 39.2 | 3.6 | 1.4 | 3.2 | | 52.6 | 8.2 | 4.8 | 10.89 | 4.6 | 0.30 |
| Work. Ex. 3 | 46.6 | 0.1 | 0.1 | | | 53.2 | 0.2 | 233.0 | 466.0 | 0.1 | 0.80 |
| Work. Ex. 4 | 40.96 | 2.23 | 2.34 | 2.12 | | 52.35 | 6.7 | 6.1 | 18.37 | 4.46 | 0.60 |
| Work. Ex. 5 | 38.4 | 1.5 | 10.1 | 6.4 | 1.2 | 42.4 | 19.2 | 2.0 | 25.60 | 17.7 | 0.40 |
| Work. Ex. 6 | 42.49 | 1.31 | 2.13 | 1.95 | | 52.12 | 5.4 | 7.9 | 32.44 | 4.08 | 0.75 |
| Work. Ex. 7 | 42.69 | 1.28 | | | | 55.93 | 1.3 | 33.4 | 33.35 | 0 | 0.70 |
| Work. Ex. 8 | 41.8 | 2.4 | 3.9 | 6.5 | | 45.4 | 12.8 | 3.3 | 17.42 | 10.4 | 0.50 |
| Comp. Ex. 1 | | 4.61 | 10.25 | 7.09 | 31 | 47.05 | 53.0 | 0.0 | 0.00 | 48.34 | 0.00 |
| Comp. Ex. 2 | 11.17 | 15.25 | 30.1 | 25.28 | 1.47 | 16.73 | 72.1 | 0.2 | 0.73 | 56.85 | 0.10 |
| Comp. Ex. 3 | 6.7 | 35.46 | 1.65 | 1.8 | 1.64 | 52.75 | 40.6 | 0.2 | 0.19 | 5.09 | 0.05 |
| Comp. Ex. 4 | 36.7 | 6.7 | 1.8 | 10.3 | | 44.5 | 18.8 | 1.95 | 5.48 | 12.1 | 0.15 |
| Comp. Ex. 5 | 9.77 | 21.54 | 11.34 | 9.51 | 1.02 | 46.82 | 43.4 | 0.2 | 0.45 | 21.87 | 0.10 |
| Comp. Ex. 6 | 8.35 | 11 | 15.18 | 13.76 | | 51.71 | 39.9 | 0.2 | 0.76 | 28.94 | 0.05 |

All of Working Examples 1 to 8, which are examples of the present invention, satisfy the relationship Al/(Cr+Ni+Si+Fe)≥2.0 in atomic % ratio. Furthermore, they satisfy the relationship Al/Cr≥10. On the other hand, Comparative Example 1 contains no Al in the matrix, and therefore, no aluminum oxide is formed and both Al/(Cr+Ni+Si+Fe) and Al/Cr are zero.

Moreover, all of Comparative Examples 2 to 6 satisfy the relationships Al/(Cr+Ni+Si+Fe)<2.0 and Al/Cr<10.

Furthermore, Fe+Ni+Si is 10 atm% or less in Working Examples 1 to 4, and 6 and 7, and Comparative Example 3, and more than 10 atm% in other working examples and comparative examples.

The ratio of the thickness of the concentrated-Al layer with respect to the thickness of the formed alumina barrier layer was measured in each of obtained Working Examples 1 to 8 and Comparative Examples 1 to 6. Table 3 above shows the results.

Table 3 shows that the ratio of the thickness of the concentrated-Al layer with respect to the thickness of the alumina barrier layer is 0.3 or more, that is, one fifth or more in each working example, but it is 0.15 at most in the comparative examples. It should be noted that since Comparative Example 1 contains no Al, no alumina barrier layer is formed.

This shows that since the low-temperature heat treatment was performed on the working examples, which were examples of the present invention, at a temperature of less than 1050°C and the high-temperature heat treatment was performed thereon at a temperature of 1050°C or more, the dilute-Al layer was formed on the surface of the matrix by the low-temperature heat treatment and then the concentrated-Al layer could be formed between the dilute-Al layer and the matrix by the high-temperature heat treatment.

On the other hand, it is thought that the ratio of the thickness of the concentrated-Al layer with respect to the thickness of the alumina barrier layer was 0.15 at most in Comparative Examples 2 to 6 on which the alumina barrier layer was formed for the following reasons.

In Comparative Example 2, the cast body contained Al in a small amount of 0.9%, and Al for forming a film on the surface of the cast body was insufficient. In Comparative Example 3, since the low-temperature heat treatment was performed at a high temperature of 1200°C, oxides containing Cr, Ni, Si, Fe and the like as a main component were formed before the alumina barrier layer having a γ or θ alumina structure was formed. In Comparative Example 4, since the low-temperature heat treatment was performed at a low temperature of 500°C, no alumina barrier layer having a γ or θ alumina structure was formed. In Comparative Examples 5 and 6, the high-temperature heat treatment was performed at a low temperature of 1000°C. As a result, a small amount of oxygen passed through the dilute-Al layer in the high-temperature heat treatment after the dilute-Al layer was formed in the low-temperature heat treatment, and Al did not obtain sufficient energy for binding to the oxygen taken in because the temperature was low.

Next, a coking test was performed on the obtained sample tubes.

The coking test was performed by placing the sample tubes in an electric furnace, supplying a hydrocarbon (ethane) to the sample tubes, and then heating them at a high temperature (955°C) for a predetermined time (12 to 24 hours). After the test, the degrees of carburization of the inner surfaces of the sample tubes were compared, and the weight ratio of coke (carbon) adhering to the inner surface of each sample tube was measured. Table 4 shows the results.

**Table 4**

| No. | Carburization resistance | Weight ratio of formed coke | Surface roughness (Ra) |
|---|---|---|---|
| Work. Ex. 1 | Good | 0.4 | 0.13 |
| Work. Ex. 2 | Fair | 0.6 | 5.51 |
| Work. Ex. 3 | Good | 0.8 | 7.63 |
| Work. Ex. 4 | Good | 0.6 | 1.53 |
| Work. Ex. 5 | Fair | 1.0 | 11.7 |
| Work. Ex. 6 | Good | 0.6 | 1.54 |
| Work. Ex. 7 | Good | 0.7 | 2.02 |
| Work. Ex. 8 | Good | 1.1 | 13.8 |
| Comp. Ex. 1 | Poor | 0.9 | 9.17 |
| Comp. Ex. 2 | Poor | 0.7 | 4.5 |
| Comp. Ex. 3 | Poor | 1.5 | 18.1 |
| Comp. Ex. 4 | Poor | 0.7 | 8.32 |
| Comp. Ex. 5 | Poor | 0.8 | 6.27 |
| Comp. Ex. 6 | Poor | 1.4 | 16.47 |

Table 4 shows that all of Working Examples 1 to 8, which were examples of the present invention, had favorable carburization resistance. On the other hand, all of the comparative examples were carburized to the inside of the sample tube.

It is because the alumina barrier layer having a stable α alumina structure (corundum structure) that was constituted by the concentrated-Al layer and the dilute-Al layer was preferably formed on the surface of the matrix that Working Examples 1 to 8 had superior carburization resistance. In particular, Working Examples 1, 3, 4, and 6 to 8 had extremely superior carburization resistance compared with the other working examples. It is thought that this is because a smaller amount of the concentrated-Al layer was formed in Working Examples 2 and 5 than in the other working examples.

Furthermore, the surface roughness (Ra) of each sample tube was measured. Table 4 shows the results as well. Table 4 shows that the weight ratio of the formed coke and the surface roughness (Ra) were substantially in proportion to each other. Accordingly, the surface roughness (Ra) is preferably 15 µm or less, and more preferably 10 µm or less.

It is possible to adjust the surface roughness (Ra) by performing the heat treatment while rotating the cast product. It is thought that it is because the heat treatment for forming a film was not properly performed and the surface roughness was increased due to the peeling and restoration of the film that the surface roughness of Comparative Examples 3 and 6 exceeded 15 µm.

### Example 2

The alumina barrier layers of Inventive Examples 2 and 7 are observed using a transmission electron microscope (TEM). Furthermore, the EDX analysis was performed on the dilute-Al layer and the concentrated-Al layer of each inventive example. FIG. 4 shows the results from Inventive Example 2, and FIG. 5 shows the results from Inventive Example 7.

FIG. 4 shows that in Inventive Example 2, small amounts of Cr, Fe, and Ni were detected in the dilute-Al layer 22 formed on the surface side, which contained Al oxides as a main component. On the other hand, no Cr, Fe, Ni, and the like were detected in the concentrated-Al layer 24 but Al. Accordingly, it is found that the concentrated-Al layer 24 was made of aluminum oxide having a very high purity.

FIG. 5 shows that in Inventive Example 7, a small amount of Cr was detected in the dilute-Al layer 22 formed on the surface side, which mainly included Al oxides. On the other hand, nothing but Al was detected in the concentrated-Al layer 24. Accordingly, it is found that the concentrated-Al layer 24 was made of aluminum oxide having a very high purity.

## Claims

1. A cast product having an alumina barrier layer including an aluminum oxide on a surface of a matrix,
wherein the aluminum oxide has a solid solution formed by at least one of Cr, Ni, Si, and Fe in a relationship Al/(Cr+Ni+Si+Fe)≥2.0 in an atomic % ratio, and has a corundum structure that is 80 vol% or more of a crystal structure, and
wherein the matrix includes C in an amount of 0.05 to 0.7 mass%, Si in an amount of more than 0 mass% to 2.5 mass% or less, Mn in an amount of more than 0 mass% to 3.0 mass% or less, Cr in an amount of 15.0 to 50.0 mass%, Ni in an amount of 18.0 to 70.0 mass%, Al in an amount of 1.0 to 5.0 mass%, rare earth elements in an amount of 0.005 to 0.4 mass%, and W in an amount of 0.5 to 10.0 mass% and/or Mo in an amount of 0.1 to 5.0 mass%, and the balance includes Fe and inevitable impurities,
including at least one selected from the group consisting of Ti in an amount of 0.01 to 0.6 mass%, Zr in an amount of 0.01 to 0.6 mass%, and Nb in an amount of 0.1 to 1.8 mass%, and including B in an amount of 0 mass% to 0.1 mass%.

2. The cast product according to claim 1,
wherein at least Cr forms a solid solution in the aluminum oxide, and the Cr forming the solid solution with Al is contained so as to satisfy a relationship Al/Cr≥10 in an atomic % ratio.

3. The cast product according to claim 1 or 2,
wherein at least one of Ni, Si, and Fe forms a solid solution in the aluminum oxide, and a total atomic % of the at least one of Ni, Si, and Fe forming the solid solution with Al is 10 atomic% or less.

4. The cast product according to any one of claims 1 to 3,
wherein the aluminum oxide has an Al-rich layer in which the Al/(Cr+Ni+Si+Fe) on the matrix side is larger than that on the surface side.

5. The cast product according to claim 4,
wherein a thickness of the Al-rich layer is one fifth or more of a thickness of the alumina barrier layer.

6. The cast product according to any one of claims 1 to 5,
wherein the alumina barrier layer has a surface roughness (Ra) of 15 µm or less.

7. A reaction tube made of the cast product according to any one of claims 1 to 6,
the alumina barrier layer being formed on an inner surface of the tube through which hydrocarbon gas as a raw material flows.

8. A method for producing the cast product according to any one of claims 1 to 6, the method being **characterized by** including a two-stage heat treatment process after casting, wherein a first heat treatment is conducted at a temperature in the range of 600 to 900°C for 5 to 15 hours under an oxidizing atmosphere and aluminum oxide having a metastable γ or θ alumina structure is formed in the first heat treatment, and a second heat treatment is conducted at a temperature of at least 1050°C for 3 to 15 hours under an oxidizing atmosphere, the alumina oxide having a metastable γ or θ alumina structure formed by the first heat treatment is phase-transformed into an α alumina structure in the second heat treatment and the second heat treatment is conducted until oxygen passes through the aluminum oxide layer.

## Patentansprüche

1. Gussprodukt mit einer Aluminiumoxidsperrschicht, beinhaltend ein Aluminiumoxid auf einer Oberfläche einer Matrix,
wobei das Aluminiumoxid eine feste Lösung, gebildet durch mindestens eines aus Cr, Ni, Si und Fe in einer Beziehung Al/(Cr+Ni+Si+Fe)≥2,0 in einem Atom-%-Verhältnis und eine Korundstruktur, welche 80 Vol.-% oder mehr einer Kristallstruktur ist, aufweist, und
wobei die Matrix C in einer Menge von 0,05 bis 0,7 Masse-%, Si in einer Menge von mehr als 0 Masse-% bis 2,5 Masse-% oder weniger, Mn in einer Menge von mehr als 0 Masse-% bis 3,0 Masse-% oder weniger, Cr in einer Menge von 15,0 bis 50,0 Masse-%, Ni in einer Menge von 18,0 bis 70,0 Masse-%, Al in einer Menge von 1,0 bis 5,0 Masse-%, Seltenerdelemente in einer Menge von 0,005 bis 0,4 Masse-%, und W in einer Menge von 0,5 bis 10,0 Masse-% und/oder Mo in einer Menge von 0,1 bis 5,0 Masse-%, beinhaltet, und der Rest Fe und unvermeidbare Verunreinigungen beinhaltet,
einschließlich mindestens eines, gewählt aus der Gruppe, bestehend aus Ti in einer Menge von 0,01 bis 0,6 Masse-%, Zr in einer Menge von 0,01 bis 0,6 Masse% und Nb in einer Menge von 0,1 bis 1,8 Masse-%, und einschließlich B in einer Menge von 0 Masse-% bis 0,1 Masse-%.

2. Gussprodukt nach Anspruch 1,
wobei mindestens Cr eine feste Lösung in dem Aluminiumoxid bildet, und das die mit Al die feste Lösung bildende Cr so enthalten ist, dass es der Beziehung Al/Cr≥10 als Atom-%-Verhältnis genügt.

3. Gussprodukt nach Anspruch 1 oder 2,
wobei mindestens eines von Ni, Si und Fe eine feste Lösung in dem Aluminiumoxid bildet, und ein Gesamtatom-%-Anteil des mindestens einen aus Ni, Si und Fe, das eine feste Lösung mit Al bildet, 10 Atom-% oder weniger beträgt.

4. Gussprodukt nach irgendeinem der Ansprüche 1 bis 3,
wobei das Aluminiumoxid eine Al-reiche Schicht aufweist, in welcher das Al/(Cr+Ni+Si+Fe) auf der Matrixseite größer ist als das auf der Oberflächenseite.

5. Gussprodukt nach Anspruch 4,
wobei die Dicke der Al-reichen Schicht ein Fünftel oder mehr einer Dicke der Aluminiumoxidsperrschicht beträgt.

6. Gussprodukt nach irgendeinem der Ansprüche 1 bis 5,
wobei die Aluminiumoxidsperrschicht eine Oberflächenrauigkeit (Ra) von 15 µm oder weniger aufweist.

7. Reaktionsrohr, hergestellt aus dem Gussprodukt nach irgendeinem der Ansprüche 1 bis 6,
wobei die Aluminiumoxidsperrschicht auf einer inneren Oberfläche des Rohrs gebildet ist, durch das Kohlenwasserstoffgas als ein Rohmaterial strömt.

8. Verfahren zur Herstellung des Gussprodukts nach irgendeinem der Ansprüche 1 bis 6, wobei das Verfahren **dadurch gekennzeichnet ist, dass** es ein zweistufiges Wärmebehandlungsverfahren nach dem Gießen beinhaltet, wobei eine erste Wärmebehandlung bei einer Temperatur im Bereich von 600 bis 900°C während 5 bis 15 Stunden unter einer oxidierenden Atmosphäre durchgeführt wird und Aluminiumoxid mit einer metastabilen γ- oder θ-Aluminiumoxidstruktur in der ersten Wärmebehandlung gebildet wird, und eine zweite Wärmebehandlung bei einer Temperatur von mindestens 1.050°C während 3 bis 15 Stunden unter einer oxidierenden Atmosphäre durchgeführt wird, wobei das Aluminiumoxid mit einer metastabilen γ- oder θ-Aluminiumoxidstruktur, das durch die erste Wärmebehandlung gebildet wird, in eine α-Aluminiumoxidstruktur bei der zweiten Wärmebehandlung phasentransformiert wird, und die zweite Wärmebehandlung durchgeführt wird bis Sauerstoff durch die Aluminiumoxidschicht passiert.

## Revendications

1. Produit de coulée ayant une couche barrière en alumine comprenant un oxyde d'aluminium sur une surface d'une matrice,
dans lequel l'oxyde d'aluminium a une solution solide formée par au moins l'un de Cr, Ni, Si et Fe dans une relation Al/(Cr+Ni+Si+Fe) ≥ 2,0 dans un rapport en % atomiques, et a une structure de corindon qui est de 80 % en volume ou plus d'une structure cristalline, et
dans lequel la matrice comprend C dans une quantité de 0,05 à 0,7 % en masse, Si, dans une quantité de plus de 0 % en masse à 2,5 % en masse ou moins, Mn, dans une quantité de plus de 0 % en masse à 3,0 % en masse ou moins, Cr, dans une quantité de 15,0 à 50,0 % en masse, Ni, dans une quantité de 18,0 à 70,0 % en masse, Al dans une quantité de 1,0 à 5,0 % en masse, les éléments des terres rares, dans une quantité de 0,005 à 0,4 % en masse, et W, dans une quantité de 0,5 à 10,0 % et/ou Mo, dans une quantité de 0,1 à 5,0 % en masse, et le complément comprend Fe et les impuretés inévitables,
comprenant au moins l'un choisi dans le groupe consistant en Ti dans une quantité de 0,01 à 0,6 % en masse, Zr, dans une quantité de 0,01 à 0,6 % en masse, et Nb, dans une quantité de 0,1 à 1,8 % en masse, et comprenant B dans une quantité de 0 % en masse à 0,1 % en masse.

2. Produit de coulée selon la revendication 1,
dans lequel au moins Cr forme une solution solide dans l'oxyde d'aluminium, et le Cr formant la solution solide avec Al est contenu de façon à satisfaire une relation Al/Cr ≥ 10 dans un rapport en % atomiques.

3. Produit de coulée selon l'une des revendications 1 ou 2,
dans lequel au moins l'un de Ni, Si et Fe forme une solution solide dans l'oxyde d'aluminium, et un % atomique total dudit au moins l'un de Ni, Si et Fe formant la solution solide avec Al est de 10 % atomiques ou moins.

4. Produit de coulée selon l'une quelconque des revendications 1 à 3,
dans lequel l'oxyde d'aluminium a une couche riche en Al, dans laquelle le Al/(Cr+Ni+Si+Fe) sur le côté matrice est plus grand que sur le côté surface.

5. Produit de coulée selon la revendication 4,
dans lequel une épaisseur de la couche riche en Al est un cinquième ou plus d'une épaisseur de la couche barrière en alumine.

6. Produit de coulée selon l'une quelconque des revendications 1 à 5,
dans lequel la couche barrière en alumine a une rugosité de surface (Ra) de 15 µm ou moins.

7. Tube de réaction fait du produit de coulée selon l'une quelconque des revendications 1 à 6,
la couche barrière en alumine étant formée sur une surface interne du tube à travers lequel un hydrocarbure gazeux en tant que matière première s'écoule.

8. Procédé de fabrication du produit de coulée selon l'une quelconque des revendications 1 à 6, le procédé étant **caractérisé par le fait qu'**il comprend un procédé de traitement thermique à deux stades après coulée, dans lequel un premier traitement thermique est conduit à une température dans la plage de 600 à 900°C pendant 5 à 15 heures sous une atmosphère oxydante et de l'oxyde d'aluminium ayant une structure d'alumine γ ou θ métastable est formé dans le premier traitement thermique, et un second traitement thermique est conduit à une température d'au moins 1050°C pendant 3 à 15 heures sous une atmosphère oxydante, l'oxyde d'aluminium ayant une structure d'alumine γ ou θ métastable formée par le premier traitement thermique subit une transformation de phase en une structure d'alumine α dans le second traitement thermique et le second traitement thermique est conduit jusqu'à ce que l'oxygène passe à travers la couche d'oxyde d'aluminium.
